

1

3,365,343

## LOW CARBON FORMABLE AND AGEABLE ALLOY STEELS

Milton B. Vordahl, Henderson, Nev., assignor to Crucible Steel Company of America, Pittsburgh, Pa., a corporation of New Jersey

No Drawing. Continuation-in-part of application Ser. No. 348,864, Mar. 2, 1964. This application Apr. 4, 1967, Ser. No. 628,292

3 Claims. (Cl. 75—125)

### ABSTRACT OF THE DISCLOSURE

This invention relates to alloy steels, and in particular, to alloy steels which exhibit the desirable property of being quenchable to a relatively soft condition, wherein they can be readily worked and formed, and are capable of then being heat treated by aging at a moderate temperature to yield a material of substantially greater strength and hardness. In particular, the present invention relates to steels of the above-indicated type which are low in nickel content (less than about 3.5%) and are, consequently, considerably less expensive than other steels and alloys hitherto known which exhibit the property of being quenchable to a soft condition and then hardenable to an increased strength by aging at a moderately elevated temperature.

This is a continuation-in-part of my copending application, Ser. No. 348,864, filed on Mar. 2, 1964, now abandoned.

Other age-hardenable materials are known, but none are as inexpensive as the steels of this invention. For example, the alpha-beta type titanium alloys exhibit such properties, but these are expensive materials, costing three or four dollars per pound.

Age-hardenable, fully austenitic stainless steels are known, but in these, the response to age-hardening is not ordinarily of such great magnitude as to make the steel greatly more formable in the quenched condition than it is in its age-hardened condition, and these too are relatively expensive materials, costing about sixty cents per pound or more. Age-hardenable, fully austenitic stainless steels invariably contain substantial quantities of nickel and/or manganese, for example, at least about 7½ percent of nickel or about 12 percent of manganese. They require, moreover, either careful balancing of austenite-promoting elements and ferrite-promoting elements, or small additions of an element such as phosphorus, to develop age-hardening characteristics.

There are also martensitic (such as Stainless W and Type 17-4-PH) and semi-austenitic (such as Type 17-7 PH and AM-350) stainless steels, which exhibit pronounced strengthening upon aging. However, all these require very delicately balanced compositions containing at least 4 percent of nickel or an equivalent amount of another austenite stabilizer, and all require complex cycles of heat treatment, involving such steps as double aging, sub-zero chilling, and cold working, all of which is quite incompatible with the main object of my invention, which is to afford a low-cost steel exhibiting marked response to an aging heat treatment.

Recently, there has been interest in the metallurgical arts in "maraging" steels that quench soft and are age-hardenable, but these too are relatively expensive mate-

2

rials, containing at least about 9 percent, and usually substantially more, of nickel.

I have discovered that by making steels relatively low in carbon, with a low nickel content not exceeding about 3.5 percent, together with a small amount of titanium and a small amount of aluminum and/or silicon, the balance being essentially iron, I can produce a steel that is quite inexpensive and yet exhibits the desired property of quenching to a soft condition and being age-hardenable to a condition of substantially greater strength and hardness. Such a steel is exceptionally suitable for applications requiring a low-cost alloy steel, formable, and with a reasonably good strength-to-weight ratio. The properties of my steel are suited especially for such applications as shipping containers for use in railway, motor, or air-freight transport, for structural parts of railway cars, trucks and buses, and the like.

Reference is directed to Table I, below, which illustrates the chemical composition of the steels of this invention, as exemplified in a general range and preferred ranges of the chemical composition of these steels.

TABLE I

|    | Element    | General Range                                                                                             | General Preferred Range | Narrow Preferred Range |
|----|------------|-----------------------------------------------------------------------------------------------------------|-------------------------|------------------------|
| 25 | Carbon     | 0.15% max.                                                                                                | 0.08% max.              | 0.08% max.             |
|    | Copper     | 0.5-7.5% max.                                                                                             | 0.5-6% max.             | 4-6%                   |
|    | Nickel     | 1-3.5%                                                                                                    | 1.5-3.5%                | 1.5-3.5%               |
|    | Manganese  | 0.75% max.                                                                                                | 0.75% max.              | 0.50% max.             |
| 30 | Titanium   | 0.75-4%                                                                                                   | 0.75-4%                 | 1.5-3%                 |
|    | Aluminum   | 3% max.                                                                                                   | 3% max.                 | 1-3%                   |
|    | Silicon    | 3% max.                                                                                                   | 2% max.                 | 1-2%                   |
|    | Chromium   | 18% max.                                                                                                  | 2% max.                 | 0.5% max.              |
|    | Cobalt     | 20% max.                                                                                                  | 2% max.                 | 0.5% max.              |
|    | Molybdenum | 8% max.                                                                                                   | 2% max.                 | 0.5% max.              |
|    | 3 Ni-Mn-Cu | 10-16%                                                                                                    | 10-16%                  | 10-16%                 |
| 35 | Al-St.     | 1-5%                                                                                                      | 1-3%                    | 1-3%                   |
|    | Iron       | In each case, balance, except for impurities in small amounts not detrimentally affecting the properties. |                         |                        |

40 The primary object of the invention is to obtain heat-treatment response in a steel as inexpensive as possible, and hence the emphasis herein is on the low-nickel steels. That nickel and aluminum will act together to provide strengthening on aging is known, but such a concept has never heretofore been applied to the production of low-cost, low-nickel steels such as those of this invention. Moreover, I find it advantageous, with lower nickel contents, to use added copper together with titanium and silicon toward the upper ends of the ranges stated above. The copper substitutes, to some extent, for the nickel, providing an austenitic matrix that can be transformed martensitically, while the controlled low manganese content is required to avoid brittleness and unworkability. The titanium and silicon form a compound or complex that contributes strength. Low contents of carbon are preferred, to preserve workability. At least some nickel is essential, to obtain heat-treatment response, but the use of more than about 3.5 percent is generally undesirable because of greater cost without corresponding benefits. 50 Although such elements as chromium, cobalt and molybdenum can be tolerated in the rather great amounts indicated above, any advantage obtained from adding them is generally more than offset by the increased cost.

60 The composition and properties of certain alloy steels constituting individual embodiments of my invention are set forth in the following Table II.

TABLE II

| Alloy              | C  | Cu | Ni    | Mn  | Ti    | Al    | Si    | Cr | Hardness as Quenched from 1,800° F., VHN | Hardness as Aged, VHN <sup>1</sup> | Tensile Bend Ductility, (Progressive Bend Limit) | Rolling Characteristics, Edge | Rolling Characteristics, Surface |
|--------------------|----|----|-------|-----|-------|-------|-------|----|------------------------------------------|------------------------------------|--------------------------------------------------|-------------------------------|----------------------------------|
| 167-5              | 0  | 6  | 3     | 0   | 3     | 0     | 2     | 0  | 354                                      | 604                                | 2T                                               | E                             | E                                |
| 167-8              | 0  | 6  | 2     | 1/2 | 1 1/2 | 1     | 1     | 0  | 317                                      | 575                                | 1T                                               | G                             | E                                |
| 167-13             | 0  | 4  | 4     | 0   | 3     | 0     | 2     | 0  | 335                                      | 628                                | 15T                                              | E                             | E                                |
| 178-4              | 0  | 0  | 4     | 0   | 2     | 1 1/2 | 0     | 0  | 230                                      | 503                                | 4T                                               | -----                         | -----                            |
| 178-5              | 0  | 2  | 4     | 0   | 2     | 0     | 1 1/2 | 0  | 288                                      | 568                                | 1T                                               | -----                         | -----                            |
| 178-6              | 0  | 0  | 4     | 0   | 2     | 0     | 1 1/2 | 0  | 286                                      | 435                                | 5T                                               | -----                         | -----                            |
| 178-7              | 0  | 2  | 3 1/2 | 1/2 | 2     | 0     | 1 1/2 | 0  | 299                                      | 561                                | 4T                                               | -----                         | -----                            |
| 166-4              | 0  | 6  | 6     | 0   | 3     | 0     | 2     | 0  | 361                                      | 663                                | -----                                            | E                             | E                                |
| 166-6 <sup>2</sup> | 0  | 6  | 6     | 0   | 1     | 1     | 0     | 0  | 336                                      | 604                                | 2T                                               | E                             | E                                |
| 167-1              | 0  | 0  | 6     | 0   | 3     | 2     | 0     | 0  | 333                                      | 636                                | 1/2T                                             | E                             | E                                |
| 167-2              | 0  | 0  | 6     | 0   | 3     | 0     | 2     | 0  | 333                                      | 486                                | 1/2T                                             | E                             | E                                |
| 167-3              | 0  | 6  | 6     | 0   | 3     | 2     | 0     | 0  | 383                                      | 691                                | 1/2T                                             | E                             | E                                |
| 167-4              | 0  | 6  | 6     | 0   | 1 1/2 | 1     | 0     | 0  | 299                                      | 589                                | 1/2T                                             | E                             | E                                |
| 167-7              | 0  | 6  | 6     | 0   | 1 1/2 | 1     | 1     | 0  | 309                                      | 620                                | 0T                                               | E                             | E                                |
| 167-9              | .1 | 6  | 6     | 0   | 3     | 0     | 2     | 0  | 362                                      | 673                                | -----                                            | E                             | E                                |
| 167-12             | 0  | 2  | 6     | 0   | 3     | 0     | 2     | 0  | 342                                      | 681                                | 1T                                               | E                             | E                                |
| 167-13             | 0  | 6  | 1     | 1/2 | 1 1/2 | 0     | 1     | 15 | 256                                      | 506                                | 10T                                              | E                             | E                                |

<sup>1</sup> After being water-quenched from 1,800° F. and then aged for 1 hour at 1,000° F. or 3 hours at 900° F.<sup>2</sup> Also contained 8% Co, 4% Mo.

The above data were obtained by using 30-gram, triple-vacuum-melted buttons of the indicated compositions.

similar results with other alloys not within the scope of my invention, are presented in the following Table III.

TABLE III

| Alloy  | C  | Cu | Ni | Mn | Ti    | Al | Si    | Cr | Hardness as Quenched from 1,800° F., VHN | Hardness as Aged, VHN <sup>1</sup> | Rolling Characteristics, Edge | Rolling Characteristics, Surface |         |
|--------|----|----|----|----|-------|----|-------|----|------------------------------------------|------------------------------------|-------------------------------|----------------------------------|---------|
| 161-1  | 0  | 6  | 0  | 0  | 0     | 0  | 0     | 0  | 177                                      | 184                                | E                             | E                                |         |
| 162-13 | 0  | 9  | 0  | 0  | 0     | 0  | 0     | 0  | 220                                      | 304                                | VP                            | VP                               |         |
| 162-11 | 0  | 6  | 0  | 2  | 0     | 0  | 0     | 0  | 225                                      | 291                                | P                             | P                                |         |
| 162-12 | 0  | 6  | 6  | 0  | 0     | 0  | 0     | 0  | 285                                      | 381                                | E                             | E                                |         |
| 162-10 | 0  | 6  | 0  | 0  | 2     | 3  | 0     | 0  | 300                                      | 385                                | F                             | G                                |         |
| 166-3  | 0  | 0  | 0  | 0  | 3     | 0  | 1 1/2 | 0  | 300                                      | 300                                | E                             | E                                |         |
| 166-1  | 0  | 0  | 0  | 0  | 3     | 3  | 3     | 0  | 219                                      | 284                                | E                             | G                                |         |
| 166-2  | 0  | 0  | 0  | 0  | 3     | 3  | 2     | 1  | 251                                      | 222                                | E                             | E                                |         |
| 166-3  | 0  | 6  | 0  | 0  | 3     | 0  | 2     | 0  | 256                                      | 371                                | E                             | E                                |         |
| 166-5  | 0  | 6  | 0  | 0  | 6     | 0  | 2     | 0  | 310                                      | 391                                | VP                            | VP                               |         |
| 166-7  | 0  | 3  | 0  | 0  | 3     | 3  | 0     | 2  | 0                                        | 261                                | 360                           | Brittle                          | Brittle |
| 167-10 | .1 | 6  | 0  | 0  | 3     | 0  | 2     | 0  | 276                                      | 317                                | E                             | P                                |         |
| 167-11 | .1 | 6  | 0  | 1  | 1 1/2 | 0  | 1     | 0  | 294                                      | 327                                | E                             | E                                |         |
| 167-17 | 0  | 0  | 6  | 0  | 0     | 0  | 2     | 0  | 294                                      | 327                                | E                             | E                                |         |

<sup>1</sup> After being water-quenched from 1,800° F. and then aged for 1 hour at 1,000° F. or 3 hours at 900° F.

The balance in each case was iron, and all components used in melting the buttons were of the highest purity. The buttons were rolled at about 1800° F., to a thickness of about 0.05 inch, and then cleaned by pickling in dilute nitric acid solution. In the above table, the Vickers hardnesses "as quenched from 1800° F." were determined upon specimens that had been heated to the indicated temperature for one minute, and then quenched in water. The indicated rolling characteristics, edge and surface, were determined by qualitative observation; in the table, the letter E indicates "excellent" and the letter G indicates "good."

For purposes of comparison with the above alloys, 75

From the foregoing Table III, it will be apparent that certain alloys somewhat similar in composition to those of Table II, are not within my invention as defined above in Table I, and exhibit properties considerably inferior to those steels of my invention, either as respects rolling characteristics or as respects their response to heat treatment. In Table III, P and VP indicate "poor" and "very poor," respectively, and G and E have the meanings above-indicated.

Additional data concerning the response of the steels of this invention to heat treatment are presented in the following Tables IV, V, and VI.

TABLE IV

| Alloy  | Vickers Hardness After Heat Treatment |     |     |     |     |     |
|--------|---------------------------------------|-----|-----|-----|-----|-----|
|        | 1                                     | 2   | 3   | 4   | 5   | 6   |
| 167-8  | 317                                   | 575 | 250 | 548 | 249 | 545 |
| 167-9  | 361                                   | 670 | 363 | 636 | 368 | 593 |
| 167-12 | 342                                   | 681 | 335 | 604 | 340 | 600 |
| 167-15 | 256                                   | 506 | 234 | 457 | 257 | 393 |

## Heat Treatment:

- 1=1,800° F. for 1 minute, water quench.  
 2=1,800° F. for 1 minute, water quench, age for 1 hour at 1,000° F. or 3 hours at 900° F.  
 3=1,700° F. for 1 minute, water quench.  
 4=1,700° F. for 1 minute, water quench, age for 1 hour at 1,000° F. or 3 hours at 900° F.  
 5=1,600° F. for 1 minute, water quench.  
 6=1,600° F. for 1 minute, water quench, age for 1 hour at 1,000° F. or 3 hours at 900° F.

5

to 1800° F. and then aging for about 1 to 3 hours or more at a temperature of about 1000° to 900° F.

While I have shown and described herein certain embodiments of my invention, I intend to cover as well any modification or change therein that may be made without departing from the spirit and scope of the invention.

I claim:

1. A steel consisting essentially of about: up to 0.15 percent carbon, 0.5 to 7.5 percent copper, 1 to 3.5 percent nickel, up to 0.75 percent manganese, 0.75 to 4 percent titanium, up to 3 percent aluminum, up to 3 percent silicon, up to 18 percent chromium, up to 20 percent cobalt, up to 8 percent molybdenum, the sum of triple the nickel content plus the manganese content plus the copper content being in the range 10 to 16 percent, the sum of the content of aluminum and silicon being in the range 1 to 5 percent, balance essentially iron.

10

15

TABLE V

| Alloy | Heat Treatment             |                         |                         | Hardness,<br>VHN | Yield<br>Strength<br>at 0.2%<br>Offset,<br>p.s.i.×10 <sup>-3</sup> | Ultimate<br>Tensile<br>Strength,<br>p.s.i.×10 <sup>-3</sup> | Elongation<br>in 0.5 inch,<br>percent | Reduction<br>of Area,<br>percent |
|-------|----------------------------|-------------------------|-------------------------|------------------|--------------------------------------------------------------------|-------------------------------------------------------------|---------------------------------------|----------------------------------|
|       | Solution<br>Temp.,<br>° F. | Aging<br>Time,<br>Hours | Aging<br>Temp.,<br>° F. |                  |                                                                    |                                                             |                                       |                                  |
| 166-6 | 1,800                      | 1                       | 1,100                   | 357              | 132                                                                | 157                                                         | 7                                     | 17                               |
| 166-6 | 1,800                      | 1                       | 1,100                   | 360              | 133                                                                | 161                                                         | 3                                     | 4                                |
| 166-6 | 1,700                      | 3                       | 900                     | 450              | 168                                                                | 193                                                         | 3                                     | 12                               |
| 167-4 | 1,500                      | 1                       | 1,000                   | -----            | 240                                                                | 253                                                         | 2                                     | 10                               |
| 167-5 | 1,500                      | 1                       | 1,000                   | -----            | 212                                                                | 226                                                         | 3                                     | 15                               |
| 167-7 | 1,600                      | 1                       | 1,000                   | -----            | 216                                                                | 216                                                         | Broke In Grips                        | 0                                |
| 178-7 | 1,800                      | 1                       | 1,000                   | -----            | 197                                                                | 218                                                         | 0                                     | 0                                |
| 178-7 | 1,600                      | 1                       | 1,000                   | -----            | 188                                                                | 203                                                         | 12                                    | 22                               |

TABLE VI

| Alloy | Solution<br>Temp.,<br>° F. | Aging<br>Time,<br>Hours | Aging<br>Temp.,<br>° F. | Hardness,<br>VHN |
|-------|----------------------------|-------------------------|-------------------------|------------------|
| 167-4 | 1,700                      | 0                       | -----                   | 334              |
| 167-4 | 1,700                      | 1                       | 900                     | 663              |
| 167-4 | 1,700                      | 3                       | 900                     | 638              |
| 167-4 | 1,700                      | 16                      | 900                     | 668              |
| 167-4 | 1,700                      | 1                       | 1,000                   | 658              |
| 167-4 | 1,600                      | 0                       | -----                   | 375              |
| 167-4 | 1,600                      | 1                       | 900                     | 558              |
| 167-4 | 1,600                      | 3                       | 900                     | 628              |
| 167-4 | 1,600                      | 1                       | 1,000                   | 649              |
| 167-4 | 1,600                      | 2                       | 1,000                   | 632              |

As Table IV shows, the use of a lower solution temperature causes, in general, somewhat lower hardness in the solution-treated-and-aged condition. As Table V indicates, such lower hardness values are associated with lower strength and greater ductility. Table V also indicates that high strengths (over 200,000 p.s.i. yield strength) can be obtained, even with solution temperatures as low as 1500° F. Table V also shows that with certain alloys, e.g., Alloy 178-7, a considerable improvement in ductility properties can be obtained, at the expense of some diminution in hardness and strength, by using a slightly lower solution temperature.

Table VI constitutes a study of the use of different aging times and temperatures, for two different solution temperatures (1700° F. and 1600° F.). The results indicate that the steels of my invention do not tend to soften substantially upon prolonged aging.

From the foregoing it will be seen that the steels of my invention can be heat-treated to high strength by quenching from an elevated temperature such as about 1500°

35 2. A steel consisting essentially of about: up to 0.08 percent carbon, 0.5 to 6 percent copper, 1.5 to 3.5 percent nickel, up to 0.75 percent manganese, 0.75 to 4 percent titanium, up to 3 percent aluminum, up to 2 percent silicon, up to 2 percent chromium, up to 2 percent cobalt, up to 2 percent molybdenum, the sum of triple the nickel content plus the manganese content plus the copper content being in the range 10 to 16 percent, the sum of the aluminum content plus the silicon content being in the range 1 to 3 percent, balance essentially iron.

40 3. An age-hardenable, low-cost steel consisting essentially of about: up to 0.08 percent carbon, 4 to 6 percent copper, 1.5 to 3.5 percent nickel, up to 0.50 percent manganese, 1.5 to 3 percent titanium, 1 to 3 percent aluminum, 1 to 2 percent silicon, up to 0.5 percent chromium, up to 0.5 percent cobalt, up to 0.5 percent molybdenum, the sum of triple the nickel content plus the manganese content being in the range 10 to 16 percent, the sum of the content of aluminum and silicon being in the range 1 to 3 percent, balance essentially iron.

45 55

## References Cited

## UNITED STATES PATENTS

|           |         |         |       |          |
|-----------|---------|---------|-------|----------|
| 2,482,096 | 9/1949  | Clarke  | ----- | 75-125   |
| 2,694,626 | 11/1954 | Tanczyn | ----- | 75-124   |
| 2,715,576 | 8/1955  | Payson  | ----- | 75-124   |
| 2,999,039 | 9/1961  | Lula    | ----- | 75-124 X |
| 3,108,870 | 10/1963 | Brady   | ----- | 75-124   |
| 3,251,683 | 5/1966  | Hammond | ----- | 75-128   |

60 65 DAVID L. RECK, Primary Examiner.

P. WEINSTEIN, Assistant Examiner.